

Dec. 27, 1949

2,492,651

F. J. McNAMARA  
METHOD FOR DETERMINING THE ACTIVITY  
OF METALLIC CATALYSTS  
Filed Aug. 24, 1948



FIG. 1.



FIG. 2.

INVENTOR

WITNESS:

Bob P. Kitchel.

Francis J. McNamara  
BY  
Besser and Harday  
ATTORNEYS.

## UNITED STATES PATENT OFFICE

2,492,651

METHOD FOR DETERMINING THE ACTIVITY  
OF METALLIC CATALYSTSFrancis J. McNamara, Rosemont, Pa., assignor to  
Sun Oil Company, Philadelphia, Pa., a corpora-  
tion of New Jersey

Application August 24, 1946, Serial No. 692,877

8 Claims. (Cl. 41—42)

1

This invention relates broadly to a method of measuring catalytic activity of metal surfaces and more particularly to a method of obtaining indications relative to the real surface area of metallic objects so that a maximum catalytic surface area of metallic surfaces as obtained by etching or other surface roughening processes may be indicated.

In many industrial and chemical operations it is necessary to employ a metallic catalyst whose effectiveness is generally in direct proportion to its surface area. It is known that a metallic surface of average smoothness presents an apparent surface area which may be conveniently measured in terms of square inches, centimeters or the like. It is also known, however, that such apparent surface area is not equivalent to the catalytic surface area which is determined by the molecular condition of the surface, the freedom from resistant film and the added physical surface resulting from chemical or mechanical roughening. In order to achieve greater efficiency and economy in the use of metallic catalysts it has been proposed, therefore, that the surface of such metallic catalysts be treated to increase the catalytic surface area without increasing the apparent surface area. One method of preparing the surface of a metallic catalyst is to etch the surface in an acid bath or by a controlled electrolytic process. When preparing the surface of a metallic catalyst by such etching processes, it is difficult to determine when a maximum catalytic surface is obtained beyond which a further etching will have no beneficial effect.

It is therefore a principal object of this invention to provide a simple and effective electrolytic method of obtaining an indication proportional to the real surface area to determine the maximum catalytic surface area of a metallic object as produced by etching or other surface roughening processes.

Further objects and advantages of this invention will be apparent by reference to the following specification and drawing in which:

Figure 1 is a top plan view of the electrolytic apparatus of this invention and showing schematically the electrical wiring, and

Figure 2 is a side elevation sectioned on the line 2—2 of Figure 1.

Referring to the drawings, the electrolytic apparatus is shown to comprise a glass jar 10 containing an electrolyte 11 and having metallic mounting strips 12 and 13 fastened to the lip 14 of the jar. If desired the jar may be formed

2

of plastic or other electric insulating substance that is impervious to the electrolyte. The mounting strips 12 and 13 also function as electric terminals for the electrolytic apparatus and are adapted to be connected to a source of electric current. As shown in Figure 1, mounting strip 12 is connected by the wire 15 to the negative terminal of an electric power supply such as a battery (not shown). The mounting strip 13 is connected by wire 16 in series with a current measuring device 17 and a rheostat 18 to the positive terminal of the electric power supply. A voltage measuring device 19 is connected between the two mounting strips 12 and 13. In the specific example of the invention to be described, the current measuring device is a milliammeter and the voltage measuring device is a millivoltmeter but the choice of such devices is of course determined by the magnitude of the currents and voltages to be measured.

On the inside ends of the mounting strips 12 and 13 are fastened depending spring clips 20 and 21, which, being of metal, will conduct the electrolytic current to be passed from the mounting strip 12 through the electrolyte 11 and to the mounting strip 13 when the terminals are connected as shown to a direct current source of power. The spring clips 20 and 21 enable the quick and easy attachment of the metal plates or electrodes 22 and 23.

The electrolytic apparatus as described above is in the nature of a conductivity cell. If the electrolyte 11 is comprised of a very weak acid such as for example N/32 hydrochloric acid and a source of direct current is connected to the strips 12 and 13, an electric current will flow. The amount of electric current for a given applied voltage will be determined by the conductivity of the electrolytic apparatus which in this specific example is determined by the amount and the strength of the electrolyte acid, by the physical spacing of the electrodes and by the size or area of the electrodes in contact with the electrolyte. Also variations in temperature will cause changes in current flow for a given applied voltage.

In adapting the above described electrolytic apparatus to the method of this invention it is necessary that all the above mentioned variables such as temperature, applied voltage, electrode spacing and electrolyte volume and strength be rigidly fixed to known reference values. If all of the above variables are fixed to reference values and the metal electrode 22 is selected as a standard reference electrode of fixed size and known

real surface area in contact with the electrolyte, then the amount of current flowing in the cell will be directly proportional to the surface area of electrode 23 in contact with the electrolyte. Assuming that various metallic plates of identical apparent surface area but different catalytic surface area are successively connected as the metal electrode 23, it will be found that a different electric current will be passed through the electrolyte for each different plate used and that the current will be directly proportional to the catalytic surface area of the various metallic plates tested. Thus the electrolytic apparatus used by the method of this invention as described will indicate the catalytic surface area of a metallic plate or other metal object used in catalytic processes.

As a specific example of the use of this invention, consider the following. In the defluorination of petroleum products, so-called aluminum Raschig rings are used as catalysts. The preparation of these aluminum rings preliminary to their use as a catalyst requires treatment with HCl to increase the catalytic activity. When etching such rings with 6% HCl it is difficult to determine when a maximum effective catalytically active surface is obtained, as apparently the surface is formed, gradually tears away, exposing a new surface to be etched, formed, etc. By periodically connecting the aluminum ring as the electrically connecting the aluminum ring as the electrode 23 in the apparatus of this invention and checking for a maximum current reading, an indication of the maximum effective surface can be obtained. When using the invention for this purpose, it was found that a suitable operating procedure would be to adjust the rheostat 18 to obtain an applied voltage of 0.98 volt which would give a current flow of about 24 mA. through an electrolyte of N/32 HCl when maximum real surface area for the aluminum ring was obtained. It should also be mentioned that the standard reference electrode 22, when the invention was used for this purpose, was formed of an aluminum strip of a known and fixed reference surface area both real and apparent.

It should be noted, however, that the selection of metals for the electrodes 22 and 23 is not critical so long as the variables previously mentioned are fixed to known values and the apparatus is properly calibrated against a standard or reference surface. Also the choice of electrolyte is not critical except that the electrolyte should preferably be weak so as not to attack or etch the reference electrode 22 or the subject electrode 23 during the operation of the method of this invention since such etching would change the real surface area of either the reference electrode or the electrode to be measured causing obvious difficulties.

I claim:

1. The method of determining the maximum catalytic activity of etched metallic catalysts which includes the steps of connecting an untreated sample of said metallic catalyst as one electrode of an electrolytic cell, the other electrode of said cell being fixed therein and constituting a reference electrode, applying a fixed and known voltage to the electrodes of said cell, said electrodes having a fixed spacing with relation to each other, the electrolyte of said cell being of known volume and of a limited strength to preserve the catalyst intact and pass electric current therethrough, maintaining the temperature of said cell substantially constant, and taking a

reading of the current flow through said cell as a reference; removing said catalyst sample to an etching bath, returning the sample after etching and cleaning to the electrolytic cell, taking a second reading of the current flow through said cell; repeating said etching and cleaning operation together with additional current flow readings until the maximum difference in current flow reading is obtained, the highest reading indicating the most active catalytic condition of the catalyst.

2. The method of determining the maximum catalytic activity of etched metallic catalysts which includes the steps of connecting an untreated sample of said metallic catalyst as one electrode of an electrolytic cell, the other electrode of said cell being fixed therein and constituting a reference electrode, applying a fixed and known direct current voltage to the electrodes of said cell, said electrodes having a fixed spacing with relation to each other, the electrolyte of said cell being of known volume and of a limited strength to preserve the catalyst intact and pass electric current therethrough, maintaining the temperature of said cell substantially constant, and taking a reading of the direct current flow through said cell as a reference; removing said catalyst sample to an etching bath, returning the sample after etching and cleaning to the electrolytic cell, taking a second reading of the direct current flow through said cell, repeating said etching and cleaning operation together with additional current flow readings until the maximum difference in current flow reading is obtained, the highest reading indicating the most active catalytic condition for the catalyst.

3. The method of determining the maximum catalytic activity of etched metallic catalysts which includes the steps of connecting an untreated sample of said metallic catalyst as one electrode of an electrolytic cell, the other electrode of said cell being fixed therein and constituting a reference electrode, applying a fixed and known voltage to the electrodes of said cell, said electrodes having a fixed spacing with relation to each other, the electrolyte of said cell being comprised of a known volume of hydrochloric acid having a strength in the order of N/32 to preserve the catalyst intact and pass electric current therethrough, maintaining the temperature of said cell substantially constant, and taking a reading of the current flow through said cell as a reference; removing said catalyst sample to an etching bath, returning the sample after etching and cleaning to the electrolytic cell, taking a second reading of the current flow through said cell, repeating said etching and cleaning operation together with additional current flow readings until the maximum difference in current flow reading is obtained, the highest reading indicating the most active catalytic condition for the catalyst.

4. The method of determining the maximum catalytic activity of etched metallic catalysts which includes the steps of connecting an untreated sample of said metallic catalyst as one electrode of an electrolytic cell, the other electrode of said cell being fixed therein and constituting a reference electrode, applying a fixed and known direct current voltage to the electrodes of said cell, said electrodes having a fixed spacing with relation to each other, the electrolyte of said cell being comprised of a known volume of hydrochloric acid having a strength of the order of N/32 to preserve the catalyst intact and

pass electric current therethrough, maintaining the temperature of said cell substantially constant, and taking a reading of the direct current flow through said cell as a reference; removing said catalyst sample to an etching bath, returning the sample after etching and cleaning to the electrolytic cell, taking a second reading of the direct current flow through said cell, repeating said etching and cleaning operation together with additional current flow readings until the maximum difference in current flow reading is obtained, the highest reading indicating the most active catalytic condition for the catalyst.

5. The method of determining the maximum catalytic activity of treated metallic catalysts which includes the steps of connecting an untreated sample of said metallic catalyst as one electrode of an electrolytic cell, the other electrode of said cell being fixed therein and constituting a reference electrode, applying a fixed and known voltage to the electrodes of said cell, said electrodes having a fixed spacing with relation to each other, the electrolyte of said cell being of known volume and of a limited strength to preserve the catalyst intact and pass electric current therethrough, maintaining the temperature of said cell substantially constant, and taking a reading of the current flow through said cell as a reference; removing said catalyst sample for treatment of the surface to increase the catalytic activity thereof and replacing in said cell for a second reading of the amount of current passing therethrough; repeating said treatments and current flow readings until the maximum difference in current flow from the reference reading of the untreated catalyst is obtained, the highest reading indicating the most active catalytic condition of the catalyst.

6. The method of determining the maximum catalytic activity of treated metallic catalysts which includes the steps of connecting an untreated sample of said metallic catalyst as one electrode of an electrolytic cell, the other electrode of said cell being fixed therein and constituting a reference electrode, applying a fixed and known direct current voltage to the electrodes of said cell, said electrodes having a fixed spacing with relation to each other, the electrolyte of said cell being of known volume and of a limited strength to preserve the catalyst intact and pass electric current therethrough, maintaining the temperature of said cell substantially constant; and taking a reading of the direct current flow through said cell as a reference; removing said catalyst sample for treatment of the surface to increase the catalytic activity thereof and replacing in said cell for a second reading of the amount of current passing therethrough; repeating said treatment and current flow readings until the maximum difference in current flow from the reference reading of the untreated catalyst is obtained, the highest reading indicating the most active catalytic condition of the catalyst.

7. The method of determining the maximum

catalytic activity of treated metallic catalysts which includes the steps of connecting an untreated sample of said metallic catalyst as one electrode of an electrolytic cell, the other electrode of said cell being fixed therein and constituting a reference electrode, applying a fixed and known voltage to the electrodes of said cell, said electrodes having a fixed spacing with relation to each other, the electrolyte of said cell being comprised of a known volume of hydrochloric acid, having a strength in the order of N/32 to preserve the catalyst intact and pass electric current therethrough, maintaining the temperature of said cell substantially constant, and taking a reading of the current flow through said cell as a reference; removing said catalyst sample for treatment of the surface to increase the catalytic activity thereof and replacing in said cell for a second reading of the amount of current passing therethrough, repeating said treatments and current flow readings until the maximum difference in current flow over the reference reading of the untreated catalyst sample is obtained; the highest reading indicating the most active catalytic condition of the catalyst.

8. The method of determining the maximum catalytic activity of treated metallic catalysts which includes the steps of connecting an untreated sample of said metallic catalyst as one electrode of an electrolytic cell, the other electrode of said cell being fixed therein and constituting a reference electrode, applying a fixed and known direct current voltage to the electrodes of said cell, said electrodes having a fixed spacing with relation to each other, the electrolyte of said cell being comprised of a known volume of hydrochloric acid having a strength of the order of N/32 to preserve the catalyst intact and pass electric current therethrough, maintaining the temperature of said cell substantially constant and taking a reading of the direct current flow through said cell as a reference, removing said catalyst sample for treatment of the surface to increase the catalytic activity thereof and replacing in said cell for a second reading of the amount of current passing therethrough, repeating said treatments and current flow readings until the maximum difference in current flow over the reference reading of the untreated catalyst sample is obtained; the highest reading indicating the most active catalytic condition of the catalyst.

FRANCIS J. McNAMARA.

#### REFERENCES CITED

The following references are of record in the file of this patent:

#### UNITED STATES PATENTS

| Number    | Name     | Date           |
|-----------|----------|----------------|
| 1,089,030 | Angell   | Mar. 3, 1914   |
| 1,845,231 | Browning | Feb. 16, 1932  |
| 1,910,021 | Legg     | May 23, 1933   |
| 2,211,394 | Vogel    | Aug. 13, 1940  |
| 2,260,840 | Rowe     | Oct. 28, 1941  |
| 2,358,163 | Heym     | Sept. 12, 1944 |